

## UNITED STATES PATENT OFFICE

2,192,891

PHOTOGRAPHIC DEVELOPER AND PROCESS  
OF DEVELOPMENT

Helmut Borst, Berlin-Kopenick, Germany

No Drawing. Application January 8, 1938, Serial  
No. 184,037. In Germany December 21, 1936

## 15 Claims.

(Cl. 95—88)

This invention relates to improvements in photographic developers and processes of development.

For the production of the pleasant blue-black shades of developed silver in photographic emulsions, a series of blue-black developing substances is known. These substances have, however, certain disadvantages. Thus, for example, nitrobenzimidazole has the great disadvantage of gradually decomposing in the developer and in addition of considerably retarding development. Benzotriazole which is likewise frequently employed has the unpleasant property of decomposing very rapidly in the developer so that therefore in use the blue-black developing effect of the developer very rapidly deteriorates. A disadvantageous characteristic of all hitherto known blue-black developing substances further consists in that they have a retarding effect on the development. In addition these substances are very sensitive to oxidising and reducing agents such as cannot be avoided in the development.

In accordance with the present invention all these disadvantages are avoided and in addition a better blue-black tone is produced.

In the process of this invention the exposed photographic layer is treated before or during development with a halogen-substituted amino pyridine. Developers according to the invention in solid or liquid form contain the specified substance.

As particularly suitable substances may be mentioned the salts of the halogen-substituted 35 2-aminopyridines, for example 5-iodo-2-amino-pyridine, 5-bromo-2-aminopyridine, 5-chloro-2-aminopyridine, 5-chloro-2-acetylaminopyridine, 3,5-dichloro-2-aminopyridine and 3,5-dibromo-2-aminopyridine.

Such an addition has a series of advantages, in particular easy availability, cheapness in price, great stability, which far surpasses that of all known blue-black developers, possibility of easily adjusting the blue shade to any desired strength, avoidance of violet shades, which are produced particularly in the shaded portions of the image and which lead to loss of the fine gradation of these portions, independence of the composition of the developer and others.

The application of 2,4,6-trimethylpyridine (collidine) as blue-black addition is indeed known; this addition has, however, various disadvantages, for example in comparison with the 55 3,5-dichloro-2-aminopyridine hydrochloride employed according to the invention. The latter

operates up to 10 minutes unobjectionably without fogging, whereas a corresponding developer with the addition of collidine after a time of development of 10 minutes produces considerable fogging, which moreover is produced before the end of that period.

In the case of 2,4,6-trimethylpyridine there is in addition the disadvantage that this compound is liquid and is not at all suitable for the manufacture of commercial developers on this account. On comparing the specified chlorinated compound on the other hand with the known nitrobenzimidazole it must be remarked that by means of the chlorinated compound the time of development is not prolonged and that accordingly no extension of the time of exposure is necessary. This circumstance is to be considered as a particular advantage, since in practice it is necessary to work as fast as possible. In addition it is to be observed that with the application of various developers for the production of various tone effects it is not of advantage when the times of development or exposure must be varied from those with a normal developer.

The following examples illustrate the invention.

## Examples

A developer according to the invention has the following composition:

|                                        |     |      |
|----------------------------------------|-----|------|
| Monomethyl-p-aminophenol hydrochloride | g.  | 2    |
| Hydroquinone                           | g.  | 6    |
| Anhydrous sodium sulphite              | g.  | 30   |
| Anhydrous sodium carbonate             | g.  | 30   |
| Potassium bromide                      | g.  | 0.7  |
| Water                                  | cc. | 1000 |

(1) Addition of 0.1 g. of 3,5-dichloro-2-amino-pyridine hydrochloride to this developer base.

This developer gives on development for the time necessary for the corresponding developer containing no addition, beautiful blue-black coloured brilliant pictures in which in particular the clear blue shade possesses no trace of violet. Moreover no change of the gradation is observed. Experiments have further shown that even in the case of times of development of 10 minutes such as are scarcely employed in practice no fog is produced.

(2) Addition of 0.05 g. of 5-bromo-2-amino-pyridine to the above developer base.

(3) Addition of 0.08 g. of 5-iodo-2-amino-pyridine to the above developer base.

These developers not only have no retarding

effect on the development, but rather appear to have an accelerating action.

The blue shade can also be produced in such a manner that the exposed picture shortly before development is treated in a bath which contains halogen-substituted aminopyridines in solution, and the picture thereupon produced in an ordinary developer.

Of course, many other changes and variations 10 may be made by those skilled in the art in accordance with the principles set forth herein and in the claims annexed hereto.

What I claim is:

1. In the development of photographic pictures the application to an exposed silver halide emulsion of an aqueous solution containing a developing medium for said emulsion and also containing a halogen-substituted aminopyridine.
2. Process as claimed in claim 1 in which a halogen-substituted 2-aminopyridine is employed.
3. Process as claimed in claim 1 in which a 5-halogen-2-aminopyridine is employed.
4. Process as claimed in claim 1 in which there is employed a compound taken from the 25 class consisting of 5-chloro-, 5-bromo-, and 5-iodo- substituted 2-aminopyridines.
5. Process as claimed in claim 1 in which 5-chloro-2-acetylaminopyridine is employed.
6. Process as claimed in claim 1 in which a 30 3,5-dihalogen-2-aminopyridine is employed.
7. Process as claimed in claim 1 in which 3,5-dichloro-2-aminopyridine is employed.
8. Process as claimed in claim 1 in which said

exposed emulsion is first treated with said halogenated aminopyridine and then subjected to treatment with said developing medium.

9. An article of manufacture comprising a photographic developer containing a silver halide developing agent and a halogen-substituted aminopyridine.

10. An article of manufacture comprising a photographic developer containing a silver halide developing agent and a 5-halogen-2-amino- 10 pyridine.

11. An article of manufacture comprising a photographic developer containing a silver halide developing agent and 3,5-dichloro-2-amino- 15 pyridine.

12. An article of manufacture comprising a photographic developer containing a silver halide developing agent and 3,5-dichloro-2-amino- pyridine-hydrochloride.

13. A photographic developer containing 20 monomethyl-p-aminophenol hydrochloride, hydroquinone, sodium sulphite, sodium carbonate, potassium bromide and a halogen-substituted aminopyridine.

14. A photographic developer as claimed in 25 claim 13 in which there is employed a compound taken from the class consisting of 5-chloro-, 5-bromo- and 5-iodo- substituted 2-amino-pyridines.

15. A photographic developer as claimed in 30 claim 13 containing 3,5-dichloro-2-aminopyridine as a halogen-substituted aminopyridine.

HELMUT BORST.